

Nov. 17, 1925.

1,561,650

T. H. LASHAR

ANTITARNISH COMPOSITION

Filed April 23, 1924

Fig. 1



Fig. 2



Fig. 3



Fig. 4



Fig. 5



J. Holmes Lashar

INVENTOR

Penrie Davis BY Marvin Edmunds

ATTORNEYS

## UNITED STATES PATENT OFFICE.

THOMAS HOLMES LASHAR, OF CHICAGO, ILLINOIS.

## ANTITARNISH COMPOSITION.

Application filed April 23, 1924. Serial No. 708,354.

*To all whom it may concern:*

Be it known that I, THOMAS HOLMES LASHAR, a citizen of the United States, residing at Chicago, in the county of Cook, 5 State of Illinois, have invented certain new and useful Improvements in Antitarnish Composition; and I do hereby declare the following to be a full, clear, and exact description of the invention, such as will enable others skilled in the art to which it app- 10 pertains to make and use the same.

This invention relates to improvements in the prevention of tarnish of silver and other metal articles, and includes an im- 15 proved anti-tarnish composition as well as articles and structures adapted for use in keeping silver and other metal articles from tarnishing.

The problem of preventing or overcoming 20 the tarnishing of silverware and other metal articles is one of the outstanding problems of the jewelry trade and is a problem wherever silverware and various other metal articles are exposed to the atmosphere, as they 25 are in show-windows, show-cases, and the like. Even where silverware is kept in closed show-cases, the occasional opening of the show-case for display purposes permits circulation of air from the outside into the 30 show-case, and sooner or later objectionable tarnishing of the silverware usually takes place. This objectionable tarnishing is particularly pronounced in cities and towns having a smoky atmosphere, where large 35 amounts of coal are burned, because of the sulfur-containing gases which the atmosphere contains, and for which silver and other metal articles have a special affinity. In large jewelry stores, or stores where large 40 displays of silverware are found, it is customary to assign one or more men to the work of polishing silverware to remove the tarnish therefrom. In the aggregate, the expense and the amount of work involved in 45 overcoming such objectionable tarnishing form a considerable part of the expense and labor of taking care of such silverware displays. The problem is presented in a somewhat similar manner with other metal articles, made of other metals than silver, and 50 is a problem with which the housewife is confronted wherever silverware is displayed or exposed to the air, since even the air of the home, particularly in large cities and 55 where the atmosphere is smoky, contains a

sufficient amount of sulfur-containing constituents to cause tarnishing of silverware after varying periods of time. This tarnishing of silver, etc. seems to be occasioned not by sulfur-containing compounds alone, but 60 by such compounds when moisture is also present. In a completely anhydrous atmosphere, even considerable amounts of sulfur-containing constituents in the air may be without objectionable tarnishing effect, even 65 after prolonged periods of time. Moreover, apparently sulfur-containing gases and par- 70 ticles in the air have an affinity for moisture, such that moist air, when laden with sulfur-containing gases, appears to be much more objectionable because of its tarnishing pro- 75 pensity.

Because of the heat conducting properties of metals, metal surfaces afford attractive surfaces for the condensation of moisture 75 thereon. If, for example, the air is warmer than the metal surface, the cooler metal sur- 80 face will tend to condense moisture from the air immediately adjacent to it, and there will tend to be formed an adsorbed or ab- 85 sorbed film of moisture on the metal surface. It is perhaps for this reason that sulfur- 90 containing gases are so objectionable when moisture is present, for if the moisture which is condensed on the metal surface 95 carries sulfur-containing gases which are condensed with it, these gases can then at- 100 tack the silver or other metal surface in the presence of sufficient moisture to permit the formation of a black film of silver sulfide, 105 to the formation of which objectionable tarnishing is due.

The present invention provides an im- 110 proved anti-tarnish composition, and im- 115 proved articles or structures embodying or combined with such anti-tarnish composi- 120 tion, whereby objectionable tarnishing of silver, etc. can be prevented for long periods of time, in a particularly effective manner.

It is well known that aqueous solutions of 125 different metal salts, when brought into contact with hydrogen sulfide and other sulfur-containing gases will react with the lat- 130 ter with precipitation of a metallic sulfide. When the water is removed from such solu- 135 tions, the absorbent power of the metal salts becomes of little or no value. Moreover, if water is present in considerable amount in show-cases and similar places where jewelry 140 and silverware are commonly kept on dis- 145

play, the humidity or water-vapor of the air in the show case will be increased, and danger from rusting of the fixtures or of some of the metal objects may exist.

5 In the new composition of the present invention I take advantage of the well known fact that metal salts in solution will absorb hydrogen sulfide, etc. from the air which comes in contact with them, but I avoid 10 aqueous solutions of such salts, and, instead, I use solutions of such salts in non-volatile solvents which are moreover hygroscopic and which tend to remove moisture from the air of the show-case or other place, 15 as well as the sulfur-containing compounds which the air contains.

I have found that the objections and limitations of aqueous solutions of such metal salts can be overcome, and new and advantageous results obtained, by dissolving the 20 metal salts in a non-volatile solvent such as glycerine, etc., in which the metal salt is soluble, and which itself has hygroscopic properties or an affinity for water-vapor 25 and water. The new composition of the present invention, accordingly, is a solution of a metal salt, such as lead acetate, in a non-volatile solvent, and particularly in such a solvent which has hygroscopic properties.

30 Different metal salts may be used in the composition of the invention but I have found that lead acetate is particularly effective. Other lead salts, however, can be used and even salts of other metals.

35 The solvents which are used may contain some water, but I have found it advantageous for best results to use a solvent which is free or relatively free from water, such as a polyhydric or polyhydroxy derivatives, especially glycerine, although other compounds such as glycols can be used, or even aqueous solutions of glucose. Glycerine not only has the property of dissolving lead acetate, for example, but in view of its 40 hygroscopic properties, it tends to attract moisture from the air, and, in this way, when exposed to the air, tends not only to remove sulfur compounds such as sulfurated hydrogen, but also to keep the air dry. Since the 45 particles of sulfur compounds tend to associate themselves with and to deposit on the particles of water-vapor in the atmosphere, the presence of a substance such as a glycerine solution of the metal-salts tends to draw 50 to it the particles of water-vapor with the sulfur particles attached thereto so that the sulfur particles react with the metallic salts dissolved in the glycerine to form a metallic 55 sulfide, instead of condensing on the metal 60 surface and tarnishing the metal.

The new composition, containing the metal salts dissolved in a non-volatile solvent, can be used in various ways. One advantageous application of the composition is 65 for impregnating a fabric to provide an

absorbent surface in the form of a pad, or layer, or sheet of impregnated fabric, containing the solution of the metal salt in the glycerine, which can be hung or exposed in cabinets, closets, show-cases and the like, and which will serve both to dry and to desulfurize the air in such places. 70

Instead of using a fabric, other absorbent materials can be used for absorbing and holding the composition so that the atmosphere to be protected from sulfur compounds is exposed to the impregnated materials. Absorbent materials such as kieselguhr may be used to absorb the solution. 75

I have found that compositions containing the lead acetate dissolved in glycerine are radically more effective than lead acetate when used in water solutions, where the water tends to evaporate and leave a dry residue of the lead acetate. 80

The nature and advantages of the invention will be further illustrated by the following examples and more detailed description.

One composition which I have found most satisfactory is made by dissolving lead acetate in glycerine in the proportion of about 1 lb. of lead acetate to 1 pint of glycerine without the addition of any water thereto. The dissolving of the lead acetate in the glycerine can advantageously be carried out by placing for example 5 gallons of glycerine (using either chemically pure yellow distilled glycerine or a crude glycerine) in a copper tank, heating to about 155° F., then adding the powdered lead acetate, and stirring until the lead acetate is dissolved. After the lead acetate is dissolved, the temperature of the solution can be lowered to about 130° F., but for the impregnation of fabric, etc., the temperature should not be 95 permitted to drop below about 100° F., as the solution becomes too thick to use readily if it is cooled below approximately such temperature. 100

In using such a solution for the impregnation of fabrics, a pad of felt or other fabric can be dipped in the solution while heated to a temperature above 100° F., e. g. around 130° F., and the impregnated fabric can then be passed through a 115 wringer. The pads, particularly if made of porous material such as felt, can then be hung up for a period e. g. of about 48 hours to allow the excess solution to drip off from the ends of the pads. Then by heating the 120 pads and passing them between steel rolls, the last trace of excess liquid can be removed and a relatively dry pad can be produced, although this pad will still contain the lead acetate in solution in the glycerine. 125

Instead of using glycerine alone for dissolving the lead acetate, I have also used an aqueous glycerine solution containing varying proportions of water and glycerine. 130 For example, a 25 per cent solution of glyc-

erine in water can be used, containing 1 quart of glycerine for every gallon of the mixture, and about 2½ lbs. of lead acetate can be dissolved therein. When water is used in this way, the lead acetate can be dissolved without the necessity of using such high temperatures as referred to in the preceding example.

In using such an aqueous glycerine solution for treating felt pads or fabrics, the pads can be dipped in the solution, then wrung and then dried in a blast of hot air to remove the water and leave the glycerine solution of the lead acetate impregnating the fabric.

For certain purposes, I find it more advantageous to use a still more dilute mixture, containing, for example, 1 pint of glycerine in each gallon, or even less glycerine, and 2 lbs. of acetate of lead per gallon. Such a solution can advantageously be used for treating box linings, curtains and other material which may come in direct contact with the silver. Box linings for example may be dipped in the solution, then wrung out, and then put in a rotating extractor to remove moisture, and the drying may then be completed by hot air or in a tumbling barrel heated by a hot air blast.

The composition can be used for rendering materials anti-tarnishing where they themselves contain objectionable sulfur compounds. Where, for example, paper, string and other substances, or material such as glue, which are used with silverware and tarnishable metals, are to be rendered anti-tarnishable, they may be analyzed to determine their sulfur content, and they may then be treated by the composition of the present invention to destroy their tarnishing properties, so that they can then be used without danger of causing tarnishing of the silverware or other articles with which they come in contact.

The formulæ and compositions referred to above, and the special methods of their application, are typical and illustrative of the invention. The particular proportions of the ingredients, and the nature of the formulæ, can be varied somewhat to take care of varying conditions.

Instead of using fabrics for carrying the composition, cardboard pads may sometimes be used, the pads being dipped, wrung and then placed in a wooden rack with air space and allowed to dry for a sufficient time. Where the composition contains water, and the fabric or other material is impregnated with it, the excess water can be subsequently removed by heating to a sufficient temperature for a suitable period of time.

Where the glycerine is used alone without water for dissolving the lead acetate, it may be heated to varying temperatures to pro-

mote the solution. The temperature may for example be from 130° F. to 175° F., although I have found a temperature of about 155° F. to be suitable for making a solution to be subsequently used for impregnating the fabric in the manner described.

In protecting show-cases and the like I have found it advantageous to use a felt-pad of appreciable thickness impregnated with the new composition. Other fabrics or other absorbent material can however be used, such as cotton, paper, wool, wicking, charcoal, hemp, kieselguhr, etc. Felt pads, however, have an appreciable thickness and can retain a considerable amount of the composition so that they are effective over relatively long periods of time. The felt pads may advantageously be placed in pad holders or frames so that they can be readily handled, and these frames can advantageously be attached to the under side of the shelves of the show case or cabinet so as to take up a minimum amount of room in the show-case, and so as not to interfere with the display of merchandise in the show-case. As distinguished from a dry fabric, the impregnated pad or fabric of the present invention, where it contains a considerable amount of the composition of the invention, has a somewhat moist feel, and some of the composition may be rubbed off on the hands if the fabric itself is directly handled. But by supporting the pad or fabric in a frame or holder, the frame or holder can be handled without touching the impregnated pad itself.

Instead of using pads of fabric, box-like containers can be used in which an absorbent material is treated with the composition and stored in such a way as to come in contact with the air which the container holds. Such a container may have holes in it which will allow the air to enter, so that, through these holes, the air has access to the composition and can come in contact with the treated absorbent material. Bowls containing the anti-tarnish composition of the invention can also be used together with a wick-like substance such as hemp or charcoal which will serve to present to the air an extended surface carrying the composition.

The use of the new composition of the invention when properly distributed and exposed to the atmosphere of a show case and the like, provides a novel and improved method for purifying the air of the show-case, etc. From the standpoint of air purification, it will be readily appreciated that it is not feasible in an ordinary jewelry store, where the door is being frequently opened by people entering and leaving the store, and where the show-case is being more or less frequently opened for the display of merchandise, to wash the air or purify it so

that the air contained in the store and in the show-case will have been previously purified. The present invention however enables the air to be maintained in a purified state by a novel method of purification. This method involves the combined desulfurizing and dehydrating of the air by the combined use of a metal salt or compound having an affinity for sulfur compounds and the use of a hygroscopic substance which has an affinity for moisture. In the process of the invention, accordingly, and in using the composition of the invention, the air is subjected to a combined drying and desulfurizing treatment by a composition which has an absorptive attraction for both moisture and sulfur-containing vapors. This purification of the air serves to protect the silverware and other metal articles from tarnishing because the moisture and sulfur-containing vapors which would otherwise tend to separate out on the metal surfaces are instead attracted to the hygroscopic and sulfur-compound-neutralizing composition of the invention. Since a sulfur-containing gas naturally tends to deposit on, or dissolve in, water vapor, and since the latter is in turn attracted to, and held by, the composition of the invention, particularly when distributed over the surface of a pad or other material, it may be said that the composition of the invention exerts a preferential affinity for moisture and for sulfur-containing vapors, and consequently brings about an effective removal of sulfur-vapors and of moisture from the air, and thereby protects the silverware and other metal objects from tarnishing.

The advantages of both drying the air and absorbing sulfur-containing gases, as compared with absorbing sulphur-containing gases without drying the air, or absorbing certain gases by solutions which increases the humidity of the air, will be appreciated when it is considered that dry gases such as hydrogen sulfide do not react readily with, or bring about, a tarnishing of metals, while the presence of moisture promotes such tarnishing when such sulfur-containing compounds are present. The composition of the invention may therefore be considered to prevent or retard tarnishing by keeping the air dry as well as by absorbing the objectionable sulfur-containing gases and compounds and thus protecting the metal surfaces from them.

In the commercial application of the invention, the particular form in which the composition, or articles carrying or impregnated by the composition, will be used will vary with the conditions where the composition is to be used. By coating a wood or other surface with the composition, the composition can be applied without the use of a fabric or similar absorbent. For ex-

ample, the under side of a shelf in a show-case, if adapted for holding a coating of the composition, can be painted or coated with the composition, and this composition will protect the air of the show-case and the silver articles in the show-case for considerable periods of time. A porous board of wood or other material can similarly be painted with the composition and hung up or supported in the show case. A particularly advantageous embodiment of the invention, however, is in the form of a fabric or pad supported in a suitable frame.

The application of the invention will be further illustrated by the accompanying drawings in which

Fig. 1 shows, in a conventional and diagrammatic manner, a felt pad or other absorbent material impregnated with the composition of the invention.

Fig. 2 shows such a pad supported in a frame.

Fig. 3 shows a further method of supporting such a pad.

Fig. 4 shows still a further method of supporting the pad, and

Fig. 5 illustrates a show-case with the invention embodied therein.

The pad of Figs. 1-4 may be a felt pad, dyed black for example and impregnated with the composition of the invention, for example, according to the first specific example hereinbefore given.

Figs. 2, 3 and 4 show various methods of supporting and holding the pad in a frame or support. In Fig. 2 the pad 1 is held between a top member 2 which may be a thin board or cardboard, and a bottom frame member 3 which holds the edges of the pad. In Fig. 3, the upper member 4 may be an ordinary board or cardboard and the lower member 5 is a perforated board or cardboard having perforations permitting the access of air to the impregnated pad. These members may be held together in any suitable way. In Fig. 4 the pad 1 is held between the upper member 6 and the frame member 7 and a screen 8 is provided for assisting in supporting the pad while permitting access of the air thereto.

Pads of this kind can be supported as indicated at 14, 15 and 17 in Fig. 5, attached to the under side of the shelves 12 and 13 or to the doors of the cabinet 9 having front and top glass members 10 and 11 and doors at the back for permitting access to the cabinet or show-case. A pad 16 is shown as supported in the upper portion of the show-case or cabinet, this pad being merely depending and supported at its upper end, or being a wick-like structure and having one end depending into a container containing the composition.

In such a show-case, the air within the show-case, while relatively quiscent, is never-

theless more or less in motion, while the opening of the door permits access of fresh air from outside and also serves to stir up and set in motion the air within the show-case. In such a show-case, however, the pad containing the composition of the invention will exert its hygroscopic action upon the air and will tend to keep it dry, while the metal salt in solution will be exposed in a reactive state to the air in the show-case and the sulphur-containing compounds will be attracted thereto and will be absorbed and held thereby. The hygroscopic nature of the glycerine solvent promotes the reaction

10 of the sulphur compounds contained in the air with the lead salt, both by attracting moisture which assists in the reaction, and by attracting moisture which may already have combined with and which carries the 15 sulfur-containing compounds themselves.

It will thus be seen that the present invention provides an improved composition as well as a felt pad or other absorbent material impregnated therewith or treated therewith, and structures such as show-cases, cabinets, etc. in which the composition is provided to protect the structures and particularly to protect the silverware and tarnishable metal articles therein. It will further be seen that the invention provides an improved method of making the composition as well as an improved method of using the composition and of saturating or treating fabrics and other materials therewith, and an improved method of protecting jewelry, silverware, etc. from tarnishing and for purifying the air of show-cases and other structures from sulfur-containing constituents having tarnishing propensities.

40 The novel composition of the invention, as hereinbefore pointed out, contains a metal salt such as lead acetate, dissolved in a solvent which is non-volatile and which has hygroscopic properties, which solution is used for treating or saturating or impregnating various fabrics or absorbent materials to give protective surfaces which when exposed to the air will serve to purify the air in the manner hereinbefore described.

50 I claim:

1. A new anti-tarnish composition comprising a solution of a metal salt capable of absorbing hydrogen sulfide in a hygroscopic non-volatile solvent.

55 2. A new anti-tarnish composition comprising a solution of a metal salt capable of absorbing hydrogen sulfide in a poly-hydroxy compound.

60 3. A new anti-tarnish composition comprising a solution of lead acetate in glycerine.

4. The method of making an anti-tarnish composition which comprises dissolving lead acetate in glycerine at an elevated temperature.

5. A new article or composition comprising an absorbent material carrying a solution of a metal salt capable of absorbing hydrogen sulfide in a hygroscopic organic solvent. 70

6. A new article or composition comprising an absorbent material carrying a solution of lead acetate in glycerine.

7. A fabric impregnated with a composition comprising a metal salt capable of absorbing hydrogen sulfide and a hygroscopic organic liquid. 75

8. A fabric impregnated with an anti-tarnish composition comprising lead acetate dissolved in glycerine. 80

9. An absorbent material carrying an anti-tarnish composition comprising a solution of a metal salt capable of absorbing hydrogen sulfide in a hygroscopic non-volatile solvent and a support for supporting said absorbent material so as to expose the anti-tarnish composition to the air. 85

10. A fabric impregnated with a solution of lead acetate in glycerine, said fabric having a supporting frame or support. 90

11. A show-case or similar structure having therein, exposed to the air therein, an anti-tarnish composition which is both hygroscopic and capable of absorbing sulfur-containing constituents from the air. 95

12. A show-case or similar structure for containing silverware and the like, having therein an extended surface, carrying a hygroscopic composition containing a metal salt capable of absorbing hydrogen sulfide, said composition being capable of absorbing both moisture and sulfur-containing constituents from the air. 100

13. A show-case or other structure adapted for containing silverware and the like, the interior of such structure having an extended surface in contact with the air of the show-case, which surface carries a solution of a metal salt capable of absorbing hydrogen sulfide in a hygroscopic organic solvent. 105

14. A show-case or other structure adapted for containing silverware and the like, the interior of such structure having an extended surface in contact with the air of the show-case, which surface carries a solution of lead acetate in glycerine. 115

15. A show-case or other structure adapted for containing silverware and the like, said structure having therein a fabric exposed to the air and which fabric carries a composition comprising lead acetate and glycerine, said composition being hygroscopic and capable of absorbing both moisture from the air and sulfur-containing compounds from the air. 120

16. The method of preparing an article or structure for anti-tarnish purposes, which comprises dissolving a metal salt capable of absorbing hydrogen sulfide in a poly-hydroxy organic solvent at an elevated tem- 125

perature and treating an absorbent material with the resulting solution while still at an elevated temperature.

17. The method of treating absorbent material for the production of anti-tarnish article or composition, which comprises forming a solution of a metal salt capable of absorbing hydrogen sulfide in aqueous glycerine, treating an absorbent material 10 with such solution, and drying the resulting product to remove water therefrom.

18. The method of preparing an anti-tarnish fabric which comprises treating the fabric at an elevated temperature with a 15 non-aqueous solution of lead acetate in glycerine, and removing the excess of the solution.

19. The method of preparing an anti-tarnish fabric which comprises treating the fabric with a solution of lead acetate in aqueous glycerine, and subsequently drying the fabric to remove water therefrom.

20. The method of preparing an anti-tarnish fabric which comprises dissolving lead 25 acetate in an aqueous solution of glycerine,

treating the fabric with such solution, removing the excess of such solution, and drying the fabric to remove water therefrom.

21. The method of purifying air in show-cases and similar structures for the protection of silverware and the like from tarnishing, which comprises subjecting the air in such structures to the purifying action of a hygroscopic composition containing a metal salt capable of absorbing hydrogen sulfide, said composition being adapted to absorb moisture from the air and also to absorb sulfur-containing constituents from the air. 30

22. The method of purifying the air in show-cases and the like for the protection of 40 jewelry, etc. from tarnishing, which comprises subjecting the air in such structures to the purifying action of a solution of lead acetate in glycerine, said solution being hygroscopic and absorbing moisture from the 45 air and also absorbing sulfur-containing constituents from the air.

In testimony whereof I affix my signature.

THOMAS HOLMES LASHAR